

## UNITED STATES PATENT OFFICE

2,435,946

## PROCESS FOR DECARBURIZING AUSTENITIC MANGANESE CAST IRON

Alfred Gordon Evans Robiette and Peter Francis Hancock, Erdington, Birmingham, England, assignors to Birlec Limited, Birmingham, England

No Drawing. Application June 30, 1943, Serial No. 492,948. In Great Britain February 27, 1942

4 Claims. (Cl. 148—16)

1

The present invention relates to improved iron alloys, and to a process for treating castings of austenitic white cast iron alloys, in which the principal alloying agent is manganese.

We have discovered that castings of austenitic white cast iron alloys in which the principal alloying agent is manganese may be subjected to a decarburising treatment whereby the average carbon content of such castings is decreased and a product is obtained having physical properties similar to those associated with austenitic manganese steel and/or whereby a graded structure with regard to the carbon content is developed and a product is obtained which for certain purposes may be equivalent or superior to a similar alloy of homogeneous carbon content such as austenitic manganese steel.

It is an object of the invention to provide an improved iron alloy in which the principal alloying ingredient is manganese.

It is another object of the invention to provide an improved iron alloy having a special combination of properties.

It is a further object of the invention to provide an improved iron alloy product having a wear or abrasion resistant surface and integral therewith a tough underlayer.

It is also an object of the invention to provide an iron alloy product having a surface with the wear and abrasion properties of manganese steel and having a core with the properties of manganese cast iron.

It is still another object of the invention to provide an integral iron alloy product having a hard martensitic surface supported by a tough austenitic underlayer and a core of austenitic manganese cast iron.

The invention also contemplates a process of treating castings of austenitic manganese white cast iron whereby the aforesaid iron alloys and iron alloy products are produced.

The invention further contemplates a process of treating castings of austenitic manganese white cast iron to impart to the surface thereof properties similar to those of wear or abrasion resisting manganese steel.

It is also within the contemplation of the invention to provide castings of an iron-manganese alloy having an increasing carbon content from the surface to the core and having a special combination of properties.

Other objects and advantages of the invention will become apparent to those skilled in the art from the following description.

2

In accordance with the present invention, castings of austenitic manganese white cast irons are decarburised by an agent which is relatively non-oxidising to the manganiferous austenite, but is decarburising to the carbon content. The decarburising agent may be gaseous, liquid or solid.

In carrying the invention into practice, the decarburising agent preferably consists of a gas or gaseous mixture maintained at substantially atmospheric pressure, that is to say, at a pressure of not less than half an atmosphere and not exceeding two atmospheres. The gaseous decarburising agent may be passed into the treatment chamber of a furnace to form an atmosphere which, if desired, may be recirculated by a fan. The re-circulation may be effected within the furnace itself by means of a fan or through a system which comprises the furnace and an external conduit. The re-circulation system may include means for regenerating the atmosphere by adding a controlled supply of air or other oxygen-containing gas whereby the carbon monoxide and hydrogen formed during the decarburising reaction are re-oxidised to carbon dioxide and water vapour. The system may also include a vent to prevent the setting up of excess internal pressure. Such an atmosphere should contain one or more of the constituents hydrogen, water vapour and carbon dioxide as decarburising agents; if carbon dioxide is present there should also be enough carbon monoxide present to reduce oxidation of the austenite to such a degree that the desired dimensions of the finished castings will not be detrimentally affected. Similarly the hydrogen-water vapour ratio should be such that the gas mixture is non-oxidising to the same extent. The mixture may be diluted with inert constituents such as nitrogen.

Alternatively, the decarburising agent may be in a solid or liquid form; also, instead of feeding the gaseous atmosphere to the treatment chamber, the said atmosphere may be generated within the furnace itself.

Thus, for example, the castings may be treated in contact with molten salts containing oxidising agents or giving rise to the same under the conditions of the reaction, for example by using molten barium chloride, with or without barium oxides or a mixture of sodium chloride and manganese dioxide. When treating the castings with a solid decarburising agent they may be heated in the present of iron ore with or without the addition of small amounts of carbon.

The cast alloy may be heated, in the presence of any of the above decarburising agents, to a temperature between about 700° C. and the temperature of incipient fusion of the alloy under treatment, the temperature and duration of treatment depending upon the thickness of the section of the casting and the properties desired.

When the castings are of relatively thick section, and a long decarburising treatment is necessary to produce the required average carbon content, it may be that there is an excessively deep zone of low carbon at the surface. In this case the castings may be submitted to a recarburising treatment, in a carburising atmosphere by which the carbon content of the surface zone is increased. If a thin surface zone of low carbon content is desired, a further short decarburising treatment may be given after the recarburising step.

The composition of the alloy as cast should preferably be in the range of about 9% to 25% manganese, about 2% to 6% of carbon, not more than about 2.0% of silicon, and not more than about 0.15% of phosphorus. Part of the manganese may be replaced by nickel and/or copper to such an extent that the alloy may contain up to a total of about 24% of nickel and copper. The nickel will substitute an approximately equal weight of manganese while the copper will substitute approximately half its weight of manganese. It will be understood that the expression "austenitic manganese cast irons" as used herein includes those alloys in which part of the manganese is substituted by nickel and/or copper but in which the manganese is not less than 5%. Other alloying elements such as chromium, molybdenum, titanium, tungsten and vanadium may also be present in quantities not exceeding about 5% of any one element and not exceeding about 12% in all, and it is not intended to exclude the presence of these elements in such amounts.

In a preferred application of the invention, the cast alloy is decarburised by a heat treatment in an atmosphere obtained by partially burning fuel gases such as coal gas, coke oven gas, producer gas, butane, propane or other hydrocarbons.

Thus for example when using an atmosphere produced from coal gas, having an approximate composition comprising about 45% to 48% of hydrogen, about 17% to 19% of methane, about 18% to 22% of carbon monoxide, about 2% to 4% of carbon dioxide, about 0.5% to 1% of oxygen, about 6% to 9% of nitrogen, and about 1.5% to 2.5% of illuminants, the gas is mixed with about 2½ to 3 parts of air by volume and the mixture burnt in a closed combustion chamber with or without a catalyst and the resulting products of combustion, after cooling to remove excess water vapour, have an approximate composition comprising about 14% to 8% of hydrogen, about 11% to 6% of carbon monoxide, about 6% to 9% of carbon dioxide, about 1% to 2% of water vapour, the balance being nitrogen. This gas will vary between these limits depending upon the exact gas to air ratio and upon the temperature of the combustion chamber and in regard to the water vapour content upon the temperature to which the gas is cooled. Alternatively, other methods of removing water vapour can be employed.

The following is an example of the production of an atmosphere using charcoal producer gas mixed with air. Charcoal producer gas has an approximate composition comprising about 30% to 32% of carbon monoxide, about 1% to 3% of carbon dioxide, about 2% to 4% of hydrogen, 75

about 1% of water vapour, the balance being nitrogen. This gas is mixed in the ratio of 4 parts of gas with one part of air and is burnt either in an externally-heated chamber or in the furnace chamber itself to give a gas having an approximate composition comprising about 20% of carbon monoxide, about 7.5% of carbon dioxide, about 2% of hydrogen, and about 1% of water vapour, the balance being nitrogen.

10 The process of decarburisation apparently operates in the following manner. The gaseous, liquid or solid decarburising medium is out of chemical equilibrium with the carbon content of the cast iron with the result that it absorbs carbon readily from the surface of the castings. If a gaseous medium is used containing hydrogen, water vapour or carbon dioxide, the reactions involved apparently are:



The carbon in the above reactions is represented for simplicity as elemental carbon, but in fact is mainly in the form of metallic carbides or the solution of carbon in iron known as austenite. The surface of the parts being treated rapidly tends to reach equilibrium with the gas, and this equilibrium carbon content depends upon the ratio of carburising and decarburising constituents of the gaseous mixture at the temperature of treatment. It is evident, therefore, that the final surface carbon content can be largely controlled by the gas composition. Preferably the gas composition is such that it is in equilibrium with a carbon content of between zero and 0.8% so as to get rapid carbon removal. It should be stated that the equilibria alter with the temperature in accordance with well-known chemical laws and the necessary gas composition may, therefore, vary with the temperature of treatment. Furthermore, the rate of diffusion of carbon to the surface is governed by the temperature and this is usually the limiting factor.

45 During the decarburising treatment, carbon is continuously removed from the surface of the casting by reaction with the decarburising agent, and simultaneously carbon diffuses from the centre, where the carbon content is high, to the surface, where it is low. As the treatment progresses, the depth of the decarburised zone increases, and if carried far enough will reach the centre of the section. Continuation of the treatment will cause a lowering of the carbon content at the centre, and a consequent flattening of the carbon content gradient from the centre of the surface. Theoretically, in the limit, a uniform carbon content would be obtained, of a value in equilibrium with the decarburising medium. In practice, the time required to approximate this result would be very long except in the case of thin sections. The characteristics of the carbon gradient are continually varying throughout the treatment, and these characteristics for a given thickness of section are influenced by the time and temperature of treatment, by the composition of the decarburising medium, by the original carbon content of the alloy, and by the diffusion constants of carbon in the austenite.

50 By suitable control of these factors, a carbon content gradient of any desired characteristics, within certain limits, may be produced. Preferably, in practice, the decarburised castings have a graded carbon content increasing from

a value in the range of 0.05% to 0.9% at the surface, to a value in the range of 0.9% to 6.0% at the core.

The metallurgical structure and the physical properties of an alloy containing manganese in the contents specified, together with the other elements, will depend upon the carbon content. It is evident, therefore, that a range of metallurgical structures can be produced from the surface to the core of the section thus treated. For example, after treatment and quenching of a casting from a temperature of approximately 1000° to 1100° C., the core may consist of a structure substantially similar to that in the original alloy, namely, carbide set in a matrix of austenite. This core will merge into an intermediate zone of substantially pure austenite, the depth or thickness of this zone depending upon the content of austenite forming elements such as manganese, nickel or copper and the time of treatment. Then, approaching the surface there will be a zone of martensite plus austenite, and with certain compositions a zone of pure martensite on the surface.

In putting the process into commercial production, normally it is found that there is formed a very thin surface skin of ferrite and/or oxide generally of a few thousandths of an inch in thickness. This, for commercial purposes can be disregarded and is incidental to the process and the product. It should, therefore, be understood that, when we refer to surface zones, we mean zones immediately underlying said thin skin of ferrite and/or oxide.

The physical characteristics of such a section would be somewhat as follows: The core would be of moderate strength and would possess low ductility, but would be supported by a tough ductile band of austenite of considerable thickness. The majority of this band would be of relatively stable austenite if quenched from a high temperature of the order of about 1000° to 1100° C. This austenite would become more unstable towards the surface where it merges into the hard martensite. This martensitic surface is brittle, but is backed by the said tough austenitic band. The resulting article as a whole will have a hard wear-resisting surface with a high rate of work hardening, a tough, strong "body" or intermediate band and a core which is moderately strong, but not ductile. The relative thickness of these bands or zones can be adjusted by the time and temperature of treatment and by control of the atmosphere during the various stages of treatment and they will also vary with the thickness of section. In thin sections the original core structure may be completely removed and the tough austenite structure can extend right to the centre.

The complex structure resulting from treatment in accordance with the present invention may have a possible application in the manufacture of armour plating, whilst for other purposes it would give rise to ideal wear and abrasion resisting properties combined with adequate strength and ductility. The resulting product is moreover cheaply and simply produced from an alloy cast iron which can be readily melted and cast by any of the well-known methods at present in use for cast and malleable irons.

The process of the invention may be applied to any type of castings. Such castings may include those made by a centrifugal process which are usually of hollow cylindrical shape; after treatment in accordance with the present invention,

such castings could be slit longitudinally and rolled, forged, or otherwise manipulated.

If it is desirable that the surface layer of any part or parts of a casting should retain its high carbon content, such part or parts may be protected from the action of the decarburising agent by any known process for protecting surfaces, such as by applying an impermeable coating of enamel or metallic deposit.

The process of the present invention enables products to be produced having a wear resistant surface zone containing at least one of the constituents austenite and martensite and a tough underlying zone or layer containing at least one of the constituents austenite and carbide. The products preferably have ultimate tensile strengths lying between 18 and 45 tons/sq. in., elongations on two inches between 8 and 35% and surface hardnesses between 200 and 400 V. P. N. with a high rate of work hardening. The tensile and elongation figures are a measure of strength and ductility of the material as a whole, and the capacity for work hardening and surface hardness are a measure of the wear resistance of the material.

Material required to have primarily high wear resistance would have analysis and treatment to give the highest obtainable surface hardness and capacity for work hardening, whereas for toughness, the analysis and treatment would aim at the optimum tensile and elongation figures.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

Having described our invention what we claim and desire to secure by Letters Patent is:

1. A process of treating a casting of austenitic carbide white cast iron having a structure comprised of austenite and free massive carbides and containing over 2% and up to about 6% carbon, about 9% to 25% manganese, and the balance essentially iron which comprises decarburizing said casting in a solid state at substantially atmospheric pressure and above about 700° C. with a gaseous decarburizing medium which is substantially non-oxidizing to the manganese austenite in said casting but is decarburizing to the carbon therein and which contains about 8% to 14% hydrogen, about 1% to 2% water vapor, about 6% to 9% carbon dioxide, about 6% to 11% carbon monoxide and the balance nitrogen, continuing said decarburizing treatment for a period of time sufficient to reduce the carbon content throughout the entire thickness of the casting and to produce a graded carbon content increasing toward the core and comprised when quenched of a work hardenable surface zone having a carbon content of less than 0.9% and a structure containing martensite on an underlayer comprised of unstable austenite merging into a deeper tough core of more stable austenite from which all free massive carbides have been removed, and quenching said casting having said graded carbon content from approximately 1000° to 1100° C.

2. A process of treating a casting of austenitic carbide white cast iron having a structure comprised of austenite and free massive carbides and containing over 2% and up to about 6% carbon,

about 9% to 25% manganese and the balance essentially iron which comprises decarburizing said casting in a solid state at substantially atmospheric pressure and above about 700° C. with a gaseous decarburizing medium which is substantially non-oxidizing to the manganiferous austenite in said casting but is decarburizing to the carbon therein, continuing said decarburizing treatment for a period of time sufficient to reduce the carbon content throughout the entire thickness of the casting and to produce in the casting a graded carbon content increasing toward the core and comprised when quenched of a work hardenable surface zone having a carbon content of less than 0.9% and a structure containing martensite on an underlayer comprised of unstable austenite merging into a deeper tough core of more stable austenite from which all free massive carbides have been removed, and quenching said casting having said graded carbon content from approximately 1000° to 1100° C.

3. A process of treating a casting of austenitic-carbidic white cast iron having a structure comprised of austenite and free massive carbides and containing over 2% and up to about 6% carbon, about 5% to 25% manganese, up to a total of 24% of at least one of the elements selected from the group consisting of nickel and copper, the amount of manganese plus nickel plus one-half the copper being 9% to 25% of the composition, and the balance essentially iron which comprises decarburizing said casting in a solid state at substantially atmospheric pressure and above about 700° C. with a gaseous decarburizing medium which is substantially non-oxidizing to the manganiferous austenite in said casting but is decarburizing to the carbon therein, continuing said decarburizing treatment for a period of time sufficient to reduce the carbon content throughout the entire thickness of the casting and to produce in the casting a graded carbon content increasing toward the core and comprised when quenched of a work hardenable surface zone having a carbon content of less than 0.9% and a structure containing martensite on an underlayer comprised of unstable austenite merging into a deeper tough core of more stable austenite from which all free massive carbides have been removed, and quenching said casting having said graded carbon content from approximately 1000° to 1100° C.

4. A process of treating a casting of austenitic-carbidic white cast iron having a structure comprised of austenite and free massive carbides and

containing over 2% and up to about 6% carbon, about 9% to 25% manganese, and the balance essentially iron which comprises decarburizing said casting in a solid state at substantially atmospheric pressure and above about 700° C. with a gaseous decarburizing medium which is substantially non-oxidizing to the manganiferous austenite in said casting but is decarburizing to the carbon therein and which contains about 2% hydrogen, about 1% water vapor, about 7.5% carbon dioxide, about 20% carbon monoxide and the balance nitrogen, continuing said decarburizing treatment for a period of time sufficient to reduce the carbon content throughout the entire thickness of the casting and to produce a graded carbon content increasing toward the core and comprised when quenched of a work hardenable surface zone having a carbon content of less than 0.9% and a structure containing martensite on an underlayer comprised of unstable austenite merging into a deeper tough core of more stable austenite from which all free massive carbides have been removed, and quenching said casting having said graded carbon content from approximately 1000° to 1100° C.

ALFRED GORDON EVANS ROBIETTE  
PETER FRANCIS HANCOCK

#### REFERENCES CITED

The following references are of record in the file of this patent:

#### UNITED STATES PATENTS

| Number    | Name      | Date          |
|-----------|-----------|---------------|
| 513,163   | Washburn  | Jan. 23, 1894 |
| 2,133,532 | Boegehold | Oct. 18, 1938 |
| 2,225,968 | Boegehold | Dec. 24, 1940 |
| 1,123,193 | Howe      | Dec. 29, 1914 |
| 2,326,838 | Crafts    | Aug. 17, 1943 |
| 1,647,096 | Jacobs    | Oct. 25, 1927 |

#### FOREIGN PATENTS

| Number  | Country              | Date          |
|---------|----------------------|---------------|
| 23,312  | Great Britain (1892) | Oct. 21, 1893 |
| 131     | Great Britain (1852) | Oct. 1, 1852  |
| 187,130 | Great Britain        | Oct. 16, 1922 |
| 419,057 | Great Britain        | Oct. 31, 1934 |
| 10,785  | Great Britain (1897) | Apr. 9, 1898  |

#### OTHER REFERENCES

"Alloy Cast Irons," Am. Foundrymen's Assoc., 1938, page 16.

"Revue de Metallurgie," July 1936, pp. 466-472.